

# UNITED STATES PATENT OFFICE.

THOMAS E. SPERRY, OF OKLAHOMA, OKLAHOMA, ASSIGNOR TO JAMES J. WALSH, OF CHICAGO, ILLINOIS.

## PATCHING CLOTH.

1,116,748.

Specification of Letters Patent. Patented Nov. 10, 1914.

No Drawing.

Application filed July 5, 1913. Serial No. 777,544.

To all whom it may concern:

Be it known that I, THOMAS E. SPERRY, a citizen of the United States, residing at Oklahoma, in the county of Oklahoma and 5 State of Oklahoma, have invented a new and useful Improvement in Patching Cloth, of which the following is a specification.

My invention relates to an improvement in the art of patching cloth, which I have 10 devised, more particularly, for patching holes and rents in the cloth on pool and billiard tables; but I do not wish to be understood as intending to limit my invention to that particular purpose, though for explaining it, the following description is mainly confined to its application thereto.

The object of my invention is to provide an invisible or seamless and durable patch covering a hole or rent that has been worn 20 or torn in cloth.

The "spot" ball on a pool-table soon wears (within a very few weeks on a much-used table) a hole in the cloth; and a mis-cue, in playing pool or billiards, is liable to tear the 25 cloth, requiring the table, to prevent unevennesses in its surface and unsightliness in its appearance, to be re-covered at considerable expense.

To employ my improvement in patching 30 a hole in the cloth of a pool or billiard table, I prepare the hole, if necessary to true it, by shearing or cutting off the frayed edges to straighten them. Thereupon a piece, of 35 suitable shape and dimensions, of adhesive fabric, which may be the material known as mending-tissue with thin-paper, or the like, covering and adhering to one surface, or a piece of very thin fabric coated with cement on one surface, is inserted underneath the 40 edges about the hole, with its cement surface against the cloth. Heat and pressure are then applied over the covered hole, as through the medium of a heated sad-iron, to effect thorough adhesion, upon cooling, of 45 the underlay or base to the cloth and hold the edges in place. This forms a shallow pocket for the filling to form the patch. Into this pocket a cementitious liquid or 50 semi-liquid compound is introduced upon the base. The preferred compound for the purpose is rubber cement (about 2 parts) and carbon bi-sulfid (about 1 part) with enough gasoline to dissolve the rubber. The carbon bi-sulfid ingredient thins the 55 cement and prevents its spreading over the

edges of the hole being patched. Upon the cementitious compound thus introduced into the pocket, fibers of cloth of the same color and preferably of the same kind of cloth as that being patched, and with the fibers by 60 preference ground up into a fine condition, are filled into the pocket, as through the medium of an adequately stiff brush. These fibers are tamped to thoroughly press them into the compound, and the whole is then 65 rolled, by means of a suitable roller, whereupon heat and pressure, (through the preferred medium of the aforesaid iron) are applied to the patch to set the material forming it. Upon cooling, the patch is perfected. It is 70 seamless and invisible, because in the use of the table the contrast in freshness of color between the newly-laid cloth fibers and the remaining surface of the cloth soon disappears.

It is preferable, in making the patch, instead of filling into the pocket the entire amount of the compound at once, and introducing thereon all of the cloth fibers required, to use only a portion of that quantity 80 of the compound at first, to introduce thereon a portion of the cloth fiber, and then tamp it down; and to repeat these successive operations as often as required to fill the pocket before applying the heat and pressure to fix and smoothen the patch and render it flush with the surface of the cloth about the hole.

I realize that considerable variation is 90 possible in the details thus specifically described, and I do not intend by thus setting forth a single, specific or preferred manner of practising an embodiment of my invention to be limited thereto; my intention being in the appended claims to claim protection upon all the novelty there may be in 95 my invention as broadly as the state of the art will permit.

What I claim as new and desire to secure 100 by Letters Patent is—

1. The method of patching cloth which consists in placing a layer of moisture resisting material across the hole to be patched forming a base beneath said hole, then inserting into the pocket thus formed a cementitious compound, then adding finely ground cloth fibers similar in nature to the material to be patched until the hole is filled with the cementitious fibrous mass, and then 105 subjecting the mixture of cementitious com- 110

pound and fibers to heat and pressure to compact and fix it and render the mass flush with the cloth surface, whereby a new piece of cloth is formed in said pocket, substantially as described.

2. The method of patching cloth which consists in placing a layer of moisture resisting material across the hole to be patched forming a base beneath the hole, then inserting into the pocket thus formed a cementitious compound containing rubber, then adding finely ground cloth fibers until the hole is filled with a cementitious fibrous mass, then subjecting the filling to heat and pressure to compact and fix it and render the patch flush with the cloth surface, whereby a new piece of cloth is formed in said pocket, substantially as described.

3. The method of patching cloth which consists in placing a layer of moisture proof material across the hole to constitute a base beneath the hole, then introducing into the pocket thus formed a cementitious compound, then adding finely ground cloth fibers of a nature similar to the cloth to be patched and repeating said introductions of cementitious compound and ground fibers until the pocket is filled with a cementitious fibrous composition, then tamping the filling and subjecting it to heat and pressure to compact and fix it and render the patch flush with the cloth surface, whereby a new piece of cloth is formed in said pocket, substantially as described.

4. The method of patching cloth which consists in fixing a piece of material to the cloth to be patched in position to extend across the hole and form a pocket, then introducing a filling of cementitious compound into the pocket, then introducing finely ground fibers of a cloth of a color to match that of the patched cloth until the pocket is filled with a cementitious fibrous substance, then compacting and forming said filling to render it flush with an outer surface of the cloth, whereby a new piece of cloth is formed in said pocket, substantially as described.

5. The method of patching the cloth of a billiard, pool or other table consisting in fixing a piece of material to the cloth to be patched in position to extend across the hole and form a pocket, then introducing into said pocket a cementitious composition formed of a compound of rubber, cement, carbon bi-sulfid, and gasoline, then adding finely ground fibers of a cloth of a color to match that of the patched cloth until the pocket is filled with a cementitious fibrous substance, then compacting and forming said filling to render it flush with a surface of the cloth, whereby a new piece of cloth is formed in said pocket, substantially as described.

THOMAS E. SPERRY.

In presence of—

NELLIE B. DEARBORN,  
OTTILIE C. AVISUS.

---

Copies of this patent may be obtained for five cents each, by addressing the "Commissioner of Patents, Washington, D. C."